

## UNITED STATES PATENT OFFICE.

SHOICHI HATTORI AND TERUZO TSUBOI, OF TOYOTAMA-GUN, TOKYO-FU, AND ITARO HORIUCHI, OF KANDA-KU, TOKYO, JAPAN.

## METHOD OF CONSTRUCTING A PROTECTIVE COATING FOR MERCHANT OR WAR SHIPS.

No Drawing.

Application filed March 4, 1922. Serial No. 541,227.

To all whom it may concern:

Be it known that we, SHOICHI HATTORI, TERUZO TSUBOI, and ITARO HORIUCHI, subjects of the Emperor of Japan, residing at

5 No. 182, Oaza-nishiokubo, Okubo-machi, Toyotama-gun, Tokyo-fu, and No. 75, Oaza-tsunohazu, Yodobashi-machi, Toyotama-gun, Tokyo-fu, and No. 7, Kajicho, Kanda-ku, Tokyo, Japan, respectively, have invented new and useful Improvements in

10 Methods of Constructing a Protective Coating for Merchant or War Ships, of which the following is a specification.

The present invention relates to a method 15 of constructing a protective coating over the surface of the sides and the bottom of a merchant or war ship especially below the water line, by covering the said surfaces with scales of thin, small, enameled, iron 20 plates, the edges of the plates overlapping one another at the seams and being enameled at the joints so as to form one continuous sheet of iron plate, and the object of this invention is to provide a coating over a ship's 25 bottom to protect it from the corrosive action of sea water and to prevent the sticking thereto of shell fish, etc.

To carry the invention into practice, the 30 surface of the bottom and up to the water-line of the vessel is studded with a plurality of ordinary bolts, the threaded ends of which project outwardly. Said bolts may be secured to the surface of the vessel by soldering by means of oxy-acetylene flame.

35 The entire surface is then covered with asphalt varnish. A plurality of iron plates, enameled with a composition hereinafter described, are each provided with an opening at each corner and at the center, and the

40 bolts are so disposed on the surface of the vessel that one will pass through each of said openings, the plates being preferably placed so as to overlap each other approximately five centimeters. Nuts are then screwed on

45 the bolts and tightened so as to firmly clamp the plates to the surface of the vessel. A coating of the composition above referred to

is then applied to the joints where the plates overlap and is melted by means of oxy-acetylene flame.

An example of the composition of the 50 enamel material for the iron plates is given below:—

|                  | Parts. |
|------------------|--------|
| Red lead         | 80     |
| Feldspar         | 33     |
| Silica powder    | 15     |
| Cryolite         | 5      |
| Sodium carbonate | 8      |
| Borax            | 25     |
| Arsenic oxide    | 10     |
| Copper oxide     | 7      |
| Sodium nitrate   | 6      |

These ingredients are first fused together and then pulverized into fine powder.

In the present enameling process, like the ordinary one, the first step consists in cleansing thin iron plates of a suitable size and preferably rectangular in shape with dilute sulphuric acid or by drochloric acid, to rid 70 them of their rust. The plates thus cleansed are coated with the enamel composition prepared as above described, and are subjected to heat in a furnace, and the composition melts and forms a uniform coating over the 75 plates.

The coating thus formed is not affected by the corrosive action of sea water or air; nor is it subject to attack by organisms, for even should some organisms such as shell-fish, sea 80 weed, or the like stick thereto, which will occur only very rarely, the organic acids secreted by these organisms will act upon the lead, arsenious acid, or copper contained in the coating and melt them, thus producing a 85 very strong poison which will quickly exterminate them. Thus the ship's bottom is always kept quite clean. When damage occurs, in any part, repair of that part can be easily effected, and this is indeed a valuable 90 part of the present invention.

We claim:

A protective coating for ships, comprising

a plurality of bolts secured to the surface of the ship and having their threaded ends extending outwardly, a plurality of enamelled scale plates each having a plurality of openings therethrough for the passage of some of said bolts, nuts for securing the plates on said bolts in overlapping relation to each

other, and an enamel composition fused in a continuous coating over said scale plates.

In testimony whereof we have signed our names to this specification.

SHOICHI HATTORI.  
TERUZO TSUBOI.  
ITARO HORIUCHI.